

## UNITED STATES PATENT OFFICE

MAX N. NICKOWITZ, OF FAIRFIELD, CONNECTICUT, ASSIGNOR TO E. I. DU PONT DE NEMOURS & COMPANY, OF WILMINGTON, DELAWARE, A CORPORATION OF DELAWARE

PROCESS OF TREATING CASEIN-VARNISH-FINISHED COATED FABRICS OR ARTICLES AND PRODUCT THEREOF

No Drawing.

Application filed November 23, 1927. Serial No. 235,404.

This invention relates to a process of treating casein varnish finished coated fabrics or articles and product thereof, and more particularly to casein varnish coated articles of manufacture which have been surface-treated with bromine to modify the surface qualities in various respects, as will be more fully described hereinafter.

It is an object of the invention to coat or surface-treat various articles of manufacture with casein varnish so as to modify the surface characteristics and, furthermore, to treat the said varnish with a halogen, preferably bromine, so as to modify the characteristics of the varnish, as for example, by somewhat softening it so that the resulting articles will have a smooth, velvety surface which will not scuff and which will not drag when such surfaces are rubbed or moved over each other. Another object of the invention is to increase the waterproof characteristics of the finish. A further object is to accomplish the aforesaid objects preferably without allowing the brominating or halogenating treatment to penetrate through to the rubber, as it is generally not desired to harden the rubber, the action of bromine in this respect being well known in the prior art. It is a still further object to prepare particularly pliable fabrics with a bromine-treated casein varnish surfacing and especially to do this without allowing the bromine to penetrate through to the rubber portion of the fabric, as it is known that bromine has a hardening action upon rubber and this would consequently interfere with the pliability of the fabric. Further objects will appear as the following description proceeds.

The aforesaid objects are accomplished in my invention, and, while various embodiments thereof may be made without departing from the spirit thereof, the following embodiments have been found by me to be advantageous in practice.

Accordingly, one embodiment consists in the following procedure: A bleached nain-sook cotton fabric is taken and the back of the fabric is coated with one spreader coat of a coating composition comprising: pale crepe rubber, 40 lbs.; zinc oxide, 5 lbs.; sul-

fur, 8 oz.; tetra-methyl-thiuram-disulfide accelerator, 4 oz.; carbon black, 1 lb.; Montan wax, 5 lbs.; barytes, 48 lbs. 4 oz.; totaling 100 lbs., this spreader coat being dissolved in gasoline, say, for example, about equal parts by weight. The face of the fabric is then given two spreader coats formed from the same kind of composition. The face is then calendered to a total gauge or thickness of twelve thousandths of an inch with the aforesaid composition, in this case the gasoline being left out. The face of the fabric is next dusted with magnesium carbonate as it comes off the calender, and the material is then vulcanized for one hour and thirty minutes at 240° F. The material is then varnished with a varnish made from the following stock formula:

|          |             |    |
|----------|-------------|----|
| Casein   | 8000 grams. | 55 |
| Water    | 1500 cc.    | 60 |
| Glycerin | 500 cc.     | 65 |
| Alcohol  | 8000 cc.    |    |
| Ammonia  | 700 cc.     |    |
| Formalin | 700 cc.     |    |

The varnish is made up in the following manner. Casein and water are warmed together and allowed to stand over night. Glycerin and ammonia are then added. The casein goes into solution at this point, after which the alcohol and formalin are added. Before application to the fabric, the above formula is diluted by adding one part of water to seven of this formula. The varnish is applied to the fabric at about 50° C. After the material is varnished, the varnish is treated with a 4% solution of bromine in carbon tetrachloride and the surface of the material is then neutralized by festooning in an atmosphere of ammonia. By this process, there is produced a rubberized fabric having a varnish coating, the surface of which is modified by bromine so as to produce the characteristics of velvety smoothness, absence of scuffing, resistance to water spotting, retention of pliability, and a certain amount of softening of the varnish.

Another embodiment of the invention consists in the following procedure and product:

The cotton fabric is dyed and the spreader coat on the back is, in this case, omitted.

Either one or two spreader coats of the same type of compound as described above are applied on the face of the fabric and these spreader coats are followed by a calender coat of the same compound to give the desired thickness of rubber coating. Casein varnish is applied at the calender, this varnish having the same composition and being prepared in the same manner as that in the preceding example. The material is then vulcanized by means of dry heat, and, after vulcanizing, the surface is brominated with a 4% solution of bromine in carbon tetra-chloride. The coated fabric is then festooned in an atmosphere of ammonia so that the free bromine and any hydrobromic acid that may be present may be neutralized. A product is formed by this process which is similar to the product of Example 1.

As a further embodiment, the procedure of Example 2 is followed, but with the difference that an additional coat or coats of casein varnish are put on after vulcanization but before bromination.

A still further embodiment consists in following the foregoing procedures but with the application of two or more coats of casein varnish to provide a total thickness of varnish film or coating sufficient to prevent the bromine, which is later applied, from penetrating the varnish coating and affecting the rubber underneath, such as hardening the rubber and reducing the pliability of the fabric. These two coats of varnish may be applied before vulcanization or after vulcanization, or one of them before and one after vulcanization, provided, in the event that both coats are applied after vulcanization, some method such as dusting the rubber surface is used to prevent sticking of the rubber surface to itself.

Another type material may be made by omitting the sulfur and accelerator from the compound and vulcanizing before the application of casein varnish by means of sulfur chloride. The sulfur chloride cure may be effected either by the application of sulfur chloride vapors or sulfur chloride solution to the surface of the material. The material is then varnished after neutralizing and the surface halogenized followed by neutralization.

An embossed fabric article may be manufactured by rubberizing a similar kind of fabric, as in the foregoing examples, and instead of applying varnish at the calender the material is first dusted with clay and is then embossed with a suitable pattern. After embossing, a very thin solution of a contrasting colored rubber is applied to give a two-tone effect. The material is then coated with casein varnish, vulcanized, brominated, and neutralized, as described above.

The coated fabric may also consist of a pyroxylin-coated material finished with casein varnish and subsequently brominated. It

might further consist of an oxidized linseed or Chinawood oil coating finished with casein varnish and subsequently brominated.

As a result of the foregoing processes, there are produced articles of manufacture, such as fabrics and coverings, which are provided with a casein varnish coating, surfaces of which are modified by a bromine treatment. I have found that the action of the bromine is to somewhat soften the varnish, with the result that the varnished surface has imparted to it a velvety smoothness and absence of so-called "drag", with the further quality of having a waterproof surface. By baking the varnish and subsequently brominating this film, I produce a more waterproof finish which does not spot as readily as an untreated varnished surface. While it is possible, with a very thin film of varnish, for the bromine to penetrate through to the rubber and thus harden it in accordance with the degree of penetration, I prefer to avoid this action by making the casein varnish film continuous and thick enough to prevent penetration by the bromine and thereby to retain pliability. This quality is important, for example, in making a coated fabric which is to be used as a garment, and, accordingly, draped in a suitable manner.

I prefer to use bromine, but other members of the halogen group may be employed in this invention, and I may also use halogen compounds, such as sulfur chloride and sulfur bromide.

In manufacturing the articles, the rubber is calendered on to the fabric by calender rolls in the manner known in the art, and the varnish is spread on the fabric in a known manner by the aid of a doctor blade, this operation being followed by drying, as for example, passing over steam coils and then cooling on a drum. The dusting of the clay is also accomplished by the aid of a doctor blade, and the surplus is brushed off. When brominating the casein varnish, the fabric is passed over rollers underneath a hood to remove objectionable halogen vapors, and the coating is performed by a roller partly submerged in the bromine solution.

As many apparently widely different embodiments of this invention may be made without departing from the spirit thereof, it is to be understood that I do not intend to limit myself to the specific embodiments thereof except as indicated in the appended claims.

I claim:

1. A process of superficially finishing rubber goods, which comprises applying a casein varnish coating to the rubber surface and then halogenizing the varnished surface.

2. A process of superficially finishing cured rubber goods, which comprises applying a casein varnish coating to the rubber surface

- and then halogenizing the varnished rubber surface.
3. A process of superficially finishing casein varnished rubber goods, which comprises halogenizing the varnished rubber surface.
5. A process of superficially finishing rubberized sheeting, which comprises curing the sheeting, applying a solution of casein varnish to the rubber surface, and finally halogenizing the varnished surface.
10. 5. An article of manufacture, comprising cured rubber goods having a coating of halogenized casein varnish.
6. An article of manufacture, comprising cured rubberized sheeting, the rubber surface of which is halogenized and coated with halogenized casein varnish.
15. 7. In the preparation of flexible, rubberized fabrics, those steps which comprise the application of a casein varnish coating thereto, and the treatment of such coating with a halogen.
20. 8. A process of superficially finishing rubber goods, which comprises applying to the rubber surface a coating of a coating composition comprising casein varnish and capable of being modified by halogenization, and halogenizing the composition.
25. 9. A process of superficially finishing rubber goods, which comprises applying to the rubber surface a coating of a coating composition comprising casein varnish and capable of being softened by halogenization, and halogenizing the composition.
30. 10. A process of finishing rubber goods, which comprises applying a casein varnish coating to the rubber surface, halogenizing the varnished surface, thereby modifying the surface of the same, and neutralizing the said surface.
35. 11. A process of superficially finishing articles of manufacture, comprising applying to the surface thereof a coating of a coating composition comprising casein varnish, and halogenizing the composition.
40. 12. An article of manufacture having a coating of halogenized casein varnish.
45. 13. An article of manufacture having a coating comprising baked casein varnish having halogenized surface portions.
50. 14. A process of finishing articles of manufacture comprising casein varnishing the surface, baking it, and then halogenizing the varnished surface.
5. In testimony whereof, I affix my signature.

MAX N. NICKOWITZ.

**CERTIFICATE OF CORRECTION.**

**Patent No. 1,746,162.**

**Granted February 4, 1930, to**

**MAX N. NICKOWITZ.**

**It is hereby certified that error appears in the printed specification of the above numbered patent requiring correction as follows: Page 3, line 16, claim 6, strike out the words "halogenized and"; and that the said Letters Patent should be read with this correction therein that the same may conform to the record of the case in the Patent Office.**

**Signed and sealed this 4th day of March, A. D. 1930.**

**(Seal)**

**M. J. Moore,  
Acting Commissioner of Patents.**